

[54] NON-FLAMMABLE PAPER FOR SPEAKER CONES

[75] Inventors: Masahiko Nakazawa; Shizuo Nakamura; Mutumi Nakayama, all of Tokyo, Japan

[73] Assignee: Asahi Denka Kogyo K.K., Tokyo, Japan

[22] Filed: July 17, 1974

[21] Appl. No.: 489,156

[30] Foreign Application Priority Data

July 19, 1973 Japan..... 48-81162

[52] U.S. Cl. .... 181/169; 162/159; 252/8.1

[51] Int. Cl. .... G10K 13/00; H04R 7/00

[58] Field of Search ..... 252/8.1; 162/159; 181/169, 181/170, 167

[56] References Cited

UNITED STATES PATENTS

|           |        |                     |         |
|-----------|--------|---------------------|---------|
| 1,759,387 | 5/1930 | Bateholts .....     | 181/170 |
| 2,416,447 | 2/1947 | Laughlin et al..... | 162/159 |
| 3,092,537 | 6/1963 | Brandts.....        | 162/159 |

|           |         |                    |         |
|-----------|---------|--------------------|---------|
| 3,436,494 | 4/1969  | Bozak .....        | 181/171 |
| 3,560,441 | 2/1971  | Schwarz et al..... | 252/8.1 |
| 3,624,028 | 11/1971 | Drake .....        | 252/8.1 |
| 3,738,958 | 6/1973  | Paul .....         | 252/8.1 |

Primary Examiner—Stephen J. Tomsky  
Attorney, Agent, or Firm—Woodhams, Blanchard and Flynn

[57] ABSTRACT

A non-flammable paper for speaker cones is prepared by adding (1) chlorinated polyolefin having a molecular weight of from 500 to 40,000 and a chlorine content of from 40 to 75 weight percent, or (1)' bromine-containing chlorinated polyolefin having a molecular weight of from 500 to 40,000, a chlorine content of from 10 to 30 percent by weight and a bromine content of from 60 to 80 percent by weight and (2) antimony trioxide into paper pulp. The paper for speaker cones thereby produced has a good non-flammable property, without losing good sound-reproducing characteristics because it has reduced hygroscopicity and increased metal protecting properties.

9 Claims, 2 Drawing Figures





Fig. 1

FREQUENCY (CYCLES PER SECOND)



Fig. 2

1  
NON-FLAMMABLE PAPER FOR SPEAKER CONES

## BACKGROUND OF THE INVENTION

## 1. Field of the Invention

This invention relates to a loudspeaker having a diaphragm or speaker cone made of a special non-flammable paper. Particularly, this invention relates to a paper for speaker cones having a good non-flammable property and good sound-reproducing characteristics.

This invention also Description of the Prior Art speaker cones which is capable of maintaining its strength for a long period of time because it possesses extremely reduced hygroscopic and increased metal protecting properties.

## 2. Description of the Prior Art

In the past, paper made of cellulosic fibers has been used as the material for making speaker cones because of its advantages such as its relatively low density, high Young's modulus, high propagation velocity of longitudinal waves, moderate vibration loss, etc.

However, such conventional paper is flammable and therefore speaker cones made of such paper without using additives, such as fire-retardants, are insufficient as non-flammable speaker cones now required in the world, especially in the United States.

Furthermore, since paper is hygroscopic and low in metal protecting property, changes of the humidity of the ambient air, etc. cause decreases in strength and deformation of speaker cones, thereby injuring their sound-reproducing characteristics.

In order to minimize or eliminate the above-mentioned disadvantages, much work has been done. For example, fire-retardants such as the following organic phosphorous compounds, halogenated organic compounds and inorganic compounds have been used as additives for imparting to paper a non-flammable property. Such organic phosphorous compounds include tricresyl phosphate, diphenylcresyl phosphate, diphenyloctyl phosphate, trichloroethyl phosphate, tributyl phosphate, triphenyl phosphate, tris(dichloropropyl) phosphate, tris(dibromopropyl) phosphate, chlorophosphonate, bromophosphonate, phosphorus-containing polyols and phosphonitrile chloride. Representative halogenated organic compounds are chloreindic acid, perbrominated polyols, tetrabrominated phthalic anhydride, tetrabrominated bisphenol A, tetrachlorinated phthalic anhydride, decachlorobiphenyl, chlorinated paraffin, polyvinyl chloride, polyvinylidene chloride, etc. Further, representative inorganic compounds are alkali metal or alkali earth metal salts of phosphoric acid and boric acid, etc.

However, the addition of the above-mentioned fire-retardants cannot impart a sufficient non-flammable property to paper. Moreover, these fire-retardants are hygroscopic and therefore cause variations of sound reproduction caused by the decrease in strength and the deformation of the speaker cones due to variations in ambient humidity. Similar phenomena are caused by heat applied during processing. Further, above-mentioned halogenated organic compounds are corrosive to metals and therefore cause the corrosion of the parts of speaker cones made from metals due to dehydrohalogenation.

## BRIEF DESCRIPTION OF THE DRAWING

FIG. 1 is a graph showing the relationship between the frequency and the sound intensity of speaker cones.

## 2

FIG. 2 is a sectional view of a typical conventional loudspeaker, the cone of which can be made of the special paper in accordance with this invention.

## SUMMARY OF THE INVENTION

We have discovered a non-flammable speaker cone capable of overcoming the above-mentioned disadvantages.

The speaker cone of this invention has a good non-flammable property; and it possesses good sound-reproducing characteristics.

It is an object of this invention to provide a speaker cone having a good fire-retardant property, as well as good sound-reproducing characteristics.

15 Another object of this invention is to provide a speaker cone capable of maintaining its strength for a long period of time because of its extremely reduced hygroscopicity and increased metal protecting properties.

20 The physical shape and size of the speaker cone is not critical, according to this invention. The speaker cone can be of any suitable shape and size in accordance with conventional practices in the loudspeaker art for the use of paper speaker cones or diaphragms, and the 25 invention does not pertain to any improvement in such physical features.

In order to make clear the overall construction of a typical loudspeaker, there is illustrated in FIG. 2, a prior art loudspeaker construction (U.S. Pat. No. 3 436

30 494) and illustrating the shape of one representative speaker cone. The loudspeaker comprises a housing 2 having a permanently magnetized pole piece 4 and a core 6 with a space for receiving a voice coil 8 of a cone-shaped diaphragm or speaker cone 10. The voice 35 coil 8 has electrically conductive wires 12 wound around the exterior surface thereof. The pole piece 4 and the core 6 provide a magnetic flux in the voice coil aperture 14 and AC electric signals conducted through wires 12 generate a second magnetic flux. The interaction of the two magnetic fluxes induces axial movement 40 of the voice coil to which the speaker cone 10 is attached. Speaker cone 10 is supported by a compliant annulus 13 at the top and bottom.

The speaker cone 10 can be made of the special 45 paper in accordance with this invention.

It will be understood, however, that the invention is not limited to the speaker cone of the shape illustrated in FIG. 2 and that the invention can be incorporated into speaker cones of various shapes and sizes in accordance with the conventional practice in the art of loudspeakers using paper speaker cones and diaphragms.

The speaker cone of this invention is made of cellulosic fiber paper. The paper contains as essential additive constituents uniformly distributed in the cellulosic fibers, (1) chlorinated polyolefin powder or (1)' bromine-containing chlorinated polyolefin powder and (2) antimony trioxide.

The preferred examples of chlorinated polyolefins are chlorinated polyethylene, chlorinated polypropylene and chlorinated rubber, wherein rubber means natural or synthetic rubber. Such synthetic rubber includes polyisoprene rubber, polyisobutene rubber, butyl rubber, SB rubber, polybutadiene rubber, neoprene rubber and nitrile rubber, and the most preferable is polyisoprene rubber. These chlorinated polyolefin materials such as chlorinated polyethylene, chlorinated polypropylene and chlorinated rubber are conventionally produced as follows.

A starting material of polyethylene, polypropylene or natural or synthetic rubber is dissolved in one or a mixture of two or more halogenated hydrocarbon solvents and then it is chlorinated by introducing a gas containing at least 80 volume percent of chlorine, and which can contain more than 0.1 volume percent of oxygen and/or ozone, at 10°-70°70 C, preferably 40°-60°C, in the presence of mineral acids containing water and radical initiators, whereby to form a reaction mixture containing chlorinated polyolefin having a chlorine content of from 40 to 75 weight percent. The chlorinated polyolefin powder having a molecular weight of 500 to 40,000 and preferably, a particle size of more than 300 mesh and less than 80 mesh, is obtained by steam distillation of the reaction mixture or precipitation in water. If the need arises, pulverization can be carried out after steam distillation or precipitation in order to adjust the particle size of the chlorinated polyolefin powder.

The halogenated hydrocarbon solvents used for dissolving said starting polyolefin must be inert during the chlorination step. Examples of the preferred solvents are halogenated lower aliphatic hydrocarbons such as methylene chloride, chloroform, carbon tetrachloride, trichloroethylene and tetrachloroethylene, and halogenated aromatic hydrocarbons such as monochlorobenzene and dichlorobenzene. The most preferred and practical solvent is carbon tetrachloride because of the solubility of the polyolefins therein, the ease of solvent removal after chlorination, and the closeness of its boiling point to that of the reaction temperature.

The amount of polyolefin dissolved in the halogenated hydrocarbon solvent is in the range of 1 to 20, preferably 3 to 10, percent by weight.

The preferred mineral acids are phosphoric acid, sulfuric acid, hydrochloric acid, etc. The concentration thereof in the aqueous acid solution is usually more than 0.1 N. The amount of aqueous mineral acid solution added to the solution of polyolefin in the halogenated hydrocarbon solvent is from 0.5 to 3.1, preferably 1 to 2, parts by weight, per one part by weight of polyolefin.

The addition of mineral acid to the chlorination reaction system is not always essential during the initial stage of the chlorination reaction, because the hydrogen chloride gas by-produced during the chlorination becomes dissolved in the water added at the initial stage to form aqueous hydrochloric acid solution. However, the concentration of the mineral acid aqueous solution must be more than 0.1 N during the final stage of the chlorination reaction.

Further, the radical initiators used in this reaction are nitrogen-containing compounds (azo compounds) having the following formula:



wherein R, R', R'' and R''', which can be the same or different, are alkyls having one to four carbon atoms, and X is —CN or —CO<sub>2</sub>R''', wherein R''' is alkyl having one to four carbon atoms.

Examples of preferred initiators are shown in the following formulas.



The amount of these azo compounds such as azobisiso-  
15 butyronitrile, added to the reaction system is from 0.01 to 1.0, preferably 0.1 to 0.5, percent by weight, based on the weight of said polyolefin. Furthermore, the chlorine gas used for chlorinating the polyolefins in the halogenated hydrocarbon solvents can be supplied in ad-  
20 mixture together with oxygen and/or ozone. However, the gas mixture must contain at least 80 volume percent of chlorine. The oxygen employed can be the oxygen gas industrially produced by air fractionation of gaseous mixtures of oxygen together with inert gases such as nitrogen and carbon dioxide, or air. Ozone, produced industrially for example by corona discharge, can also be used together with the chlorine gas.

The presence of oxygen and/or ozone in the gas remarkably stabilizes the chlorinated polyolefins pro-  
30 duced in the co-presence of said mineral acids and azo compounds in the reaction system.

When the oxygen and/or ozone content of the chlorine-containing gas is less than 0.1 volume percent, the stabilizing effect of oxygen on the chlorinated polyole-  
35 fin cannot be observed. However, the upper limit of the oxygen and/or ozone content of the chlorine-contain-  
ing gas is 20 volume percent in order to maintain the chlorine content of the gas high enough to highly chlorinate polyolefins from the economical point of view.  
40 The preferred range of oxygen and/or ozone content is 0.1 to 10 volume percent.

The oxygen can also be supplied in the form of air. Thus, the reaction gas can contain nitrogen as a nonre-  
active diluent, provided that the chlorine content of the  
45 gas is at least 80 volume percent.

In the case of mixing oxygen and/or ozone and/or air into chlorine, either of the following two methods can be adopted. One is to introduce into the reaction sys-  
50 tem a gas mixture obtained by introducing oxygen and/or ozone and/or air into the chlorine stream and mixing them uniformly therein. Another method is to intro-  
duce the chlorine gas, oxygen and/or ozone and/or air separately and then mix them in the reaction system.

Bromine-containing chlorinated polyolefins are also effective for the purpose of this invention. These bromine-containing chlorinated polyolefins are produced in such a way as disclosed in the Japanese Patent Publication No. 49-8952. The water suspension of the polyolefins listed above is reacted with a brominating agent and chlorine gas to give a bromine-containing chlorinated polyolefins.

The preferred example is a bromine-containing polyolefin having a chlorine content of from 10 to 30 per-  
65 cent by weight and a bromine content of from 60 to 80 percent.

In the past, powders of chlorinated polymers have been obtained by either direct pulverization of the solid polymers or the removal of solvent from solvent solu-

tions of the polymers by steam distilling, precipitating or spraying the reaction solution. The powder of chlorinated polyolefins used in this invention is obtained most preferably by removing the solvent from the reaction solution by means of steam distillation or precipitation into water. If necessary, pulverization can be carried out after said solvent removal to adjust the particle size. Chlorinated polyolefins obtained by steam distillation are macroscopically thin leaf or scale-like powders of low bulk density.

Chlorinated polyolefin powders obtained by precipitation in non-solvents, for example water, are macroscopically globular or ellipsoidal powders. These latter powders have more uniform particle sizes, compared with powders obtained by the other methods, and are, therefore, more preferable for use in this invention.

The particle size of chlorinated polyolefins in this invention is preferably more than 300 mesh size and less than 80 mesh size.

Another essential constituent present in the paper of the speaker cone, namely, (2) antimony trioxide is also employed in the form of a powder of preferably more than 300 mesh size and less than 80 mesh size. The speaker cone of this invention is prepared in the following way.

The preparation of the paper pulp fibers can be carried out in accordance with conventional techniques. These fibers are beaten with water to form a pulp, also in accordance with conventional papermaking techniques. The beaten pulp is thoroughly mixed with dyes, pigments and paper strengthening agents, and with the chlorinated polyolefins and antimony trioxide in a beater, in the same manner as is conventional for sizing paper. These additives are precipitated on the fibers by adding a precipitating and fixing agent such as aluminum sulfate, as is conventional. Further, the use of other additives such as coagulating agents is extremely effective.

The pulp-water suspension is poured into a porous mold to form a paper product in the form of a speaker cone. Then, the speaker-cone-type paper product is dried to give a speaker cone. In some cases, the speaker cone can be shaped by compression molding.

The preferred cellulosic fiber pulps used for the production of the speaker cone in this invention are bleached sulfate pulps of soft woods and hard woods and bleached or non-bleached sulfate pulps of mixtures of soft and hard woods.

The fiber concentration in the beaten pulp (water suspension of fibers) is from 0.01 to 0.1, preferably 0.03 to 0.07, percent by weight. Further, as paper strengthening agents there can be used known conventional agents, such as starch, natural gum, synthetic paste, polyacrylamide, ureaformaldehyde resins, epoxy resins, polyethylene imine, polyethylene oxide and mixtures thereof. The amount of paper strengthening agent added to the pulp is from 0.1 to 5 parts by weight, per 100 parts by weight of fibers.

The amount of chlorinated polyolefins added to the pulp is from 10 to 50, preferably 20 to 40, parts by weight, per 100 parts by weight of fibers. The preferred fixing agents are polyacryl amides, modified epoxy resins, starches, polyethylene imines, polyethylene oxides,

5 polyvinyl alcohol, ethylene-vinyl acetate copolymer, and carboxymethyl cellulose, the amount of antimony trioxide added to the pulp is from 5 to 40, preferably 10 to 30 parts by weight, per 100 parts by weight of fibers.

10 Further, the amount of fixing agent added is from 1 to 5, preferably 3 to 5, parts by weight, per 100 parts by weight of fibers.

The preferred coagulating agents are polyacryl amide, aluminum sulfate, polyaluminium chloride, 15 polyethylene imine, modified polyamide-epichlorohydrin resin, natural gum and the amount added to the pulp is from 0.01 to 0.1, preferably 0.05 to 0.08, parts by weight, per 100 parts by weight of fibers.

This invention provides a non-flammable speaker 20 cone capable of maintaining its strength for a long period of time because of its extremely reduced hygroscopicity and its improved metal protecting property.

In order to obtain the above-mentioned effects, the 25 molecular weight and the chlorine content of chlorinated polyolefins must be from 500 to 40,000 and from 40 to 75 weight percent, respectively. When these features deviate from the above-stated limited values, the objects of this invention cannot be achieved. For example, the addition of chlorinated polyolefins having 30 lower molecular weights and chlorine contents than the above-mentioned ranges does not impart sufficient non-flammability to the speaker cones, it causes stickiness of the speaker cones and a decrease of the sizing degree.

35 A preferred example of the preparation of chlorinated polyolefins, an essential constituent of this invention, is as follows:

Into a reaction vessel equipped with a stirrer, a chlorine introducing tube, a thermometer and a condenser, 40 are charged 60 parts (the term "parts" employed therein refers to parts by weight) of polyethylene (Trademark "Sumikathene G 801", melt index 20) and 1140 parts of carbon tetrachloride. After they are stirred at reflux temperature for 2-3 hours to dissolve 45 said polyethylene, 0.3 part of azobisisobutyronitrile (AIBN, 0.5 weight percent, based on polyethylene) is added and an oxygen-containing chlorine gas is introduced. When 256 parts of chlorine is introduced over a period of 7 hours, the reaction is stopped and the reaction 50 mixture is steam distilled to give chlorinated polyethylene powder (CPE-1) having a chlorine content 69.0 weight percent, a molecular weight of 3,000 and a particle size of 200 to 220 mesh. CPE-2, CPP-1, CPP-2, CR-1 and CR-2 are produced in a similar way as in the 55 production of CPE-1. Their chlorine content, molecular weight and particle size are shown in Table 1.

TABLE 1

|                         | CPE-1<br>chlorinated<br>polyethylene | CPE-2<br>chlorinated<br>polyethylene | CPP-1<br>chlorinated<br>polypropylene | CPP-2<br>chlorinated<br>polypropylene | CR-1<br>chlorinated<br>rubber | CR-2<br>chlorinated<br>rubber |
|-------------------------|--------------------------------------|--------------------------------------|---------------------------------------|---------------------------------------|-------------------------------|-------------------------------|
| Chlorine<br>content (%) | 69.0                                 | 45.8                                 | 71.0                                  | 59.5                                  | 68.5                          | 55.3                          |
| Molecular<br>weight     | 3,000                                | 21,000                               | 5,000                                 | 12,000                                | 5,000                         | 25,000                        |
| Particle<br>size (mesh) | 200-220                              | 80-100                               | 280-300                               | 100-120                               | 115-135                       | 85-105                        |

The following examples further illustrate this invention. The invention is not limited to the subjects matter of these examples.

### EXAMPLES 1 TO 6 AND COMPARATIVE EXAMPLES 1 TO 3

Speaker cones are produced in the following way.

After 100 parts of bleached sulfate fibers of soft wood is beaten, the following ingredients are added thereto to make a fiber-water suspension (fiber content 0.05 weight percent).

| Ingredients                                         | parts |
|-----------------------------------------------------|-------|
| direct black dye                                    | 3     |
| paper strengthening agent (urea-formaldehyde resin) | 3     |
| chlorinated polyolefin                              | 30    |
| antimony trioxide                                   | 20    |
| aluminum sulfate                                    | 5     |
| coagulating agent (Trademark Aquoflock)             | 0.08  |

The pulp-water suspension is poured into a porous speaker cone mold to form a cone-shaped wet paper product. Then, the paper is dried to give a speaker cone.

5 Table 2 shows the amount of each ingredient added and the non-flammability and sound-reproducing characteristics of the speaker cones produced.

As clearly shown in Table 2, speaker cones of this invention have good non-flammable property and extremely low propagation velocity, thereby contributing good directivity of the sound.

10 Further, FIG. 1 shows the relationship between the frequency and the sound pressure level of speaker cones in this invention. As clearly shown in FIG. 1, speaker cones of this invention have improved sound characteristics in the high frequency region and give a substantially flat sound pressure level in the middle frequency region.

TABLE 2

|           | fibers                                        | dye                               | Addition amount (parts)<br>paper<br>strengthening<br>agent | fire<br>retardant                                                                                                           | fixing agent                   | coagulating<br>agent           |
|-----------|-----------------------------------------------|-----------------------------------|------------------------------------------------------------|-----------------------------------------------------------------------------------------------------------------------------|--------------------------------|--------------------------------|
| Example 1 | N.B.K <sub>p</sub><br>(20°SR)<br>100<br>parts | direct<br>black<br>dye<br>3 parts | urea-<br>formaldehyde<br>resin<br>3 parts                  | CPE-1/30<br>parts<br>Sb <sub>2</sub> O <sub>3</sub> /20<br>parts<br>CPE-2<br>30/Sb <sub>2</sub> O <sub>3</sub><br>20, parts | aluminum<br>sulfate<br>5 parts | Aquoflock<br>305<br>0.08 parts |
| Example 2 | "                                             | "                                 | "                                                          | CPP-1<br>30/Sb <sub>2</sub> O <sub>3</sub><br>20, parts                                                                     | "                              | "                              |
| Example 3 | "                                             | "                                 | "                                                          | CPP-2<br>30/Sb <sub>2</sub> O <sub>3</sub><br>20, parts                                                                     | "                              | "                              |
| Example 4 | "                                             | "                                 | "                                                          | CR-1<br>30/Sb <sub>2</sub> O <sub>3</sub><br>20, parts                                                                      | "                              | "                              |
| Example 5 | "                                             | "                                 | "                                                          | CR-2<br>30/Sb <sub>2</sub> O <sub>3</sub><br>20, parts                                                                      | "                              | "                              |
| Example 6 | "                                             | "                                 | "                                                          | 30/Sb <sub>2</sub> O <sub>3</sub><br>20, parts                                                                              | "                              | "                              |

  

|           | fiber content<br>in water<br>suspension | weight/area         | oxygen index | propagation<br>velocity | frequency<br>character-<br>istics |
|-----------|-----------------------------------------|---------------------|--------------|-------------------------|-----------------------------------|
| Example 1 | 0.05%                                   | 30 g/m <sup>2</sup> | 32           | 200 m/sec               | solid line<br>in FIG. 1           |
| Example 2 | "                                       | "                   | 31           | 250 "                   |                                   |
| Example 3 | "                                       | "                   | 33           | 210 "                   |                                   |
| Example 4 | "                                       | "                   | 31           | 250 "                   |                                   |
| Example 5 | "                                       | "                   | 32           | 200 "                   |                                   |
| Example 6 | "                                       | "                   | 30           | 240 "                   |                                   |

  

|                          | Addition amount (parts)                       |                                   |                                           |                                             |                                |                                |
|--------------------------|-----------------------------------------------|-----------------------------------|-------------------------------------------|---------------------------------------------|--------------------------------|--------------------------------|
|                          | fiber                                         | dye                               | paper<br>strengthening<br>agent           | fire<br>retardant                           | fixing<br>agent                | coagulating<br>agent           |
| Comparative<br>Example 1 | N.B.K <sub>p</sub><br>(20°SR)<br>100<br>parts | direct<br>black<br>dye<br>3 parts | urea-<br>formaldehyde<br>resin<br>3 parts | phospho-<br>nitrile<br>chloride<br>50 parts | aluminum<br>sulfate<br>5 parts | Aquoflock<br>305<br>0.08 parts |
| Comparative<br>Example 2 | "                                             | "                                 | "                                         | polyvinyl<br>chloride<br>50 parts           | "                              | "                              |
| Comparative<br>Example 3 | "                                             | "                                 | "                                         | none                                        | "                              | "                              |

  

|                          | fiber content<br>in water<br>suspension | weight/area         | oxygen index | propagation<br>velocity | frequency<br>character-<br>istics |
|--------------------------|-----------------------------------------|---------------------|--------------|-------------------------|-----------------------------------|
| Comparative<br>Example 1 | 0.05%                                   | 30 g/m <sup>2</sup> | 23           | 900 m/sec               | dotted line<br>in FIG. 1          |
| Comparative<br>Example 2 | "                                       | "                   | 21           | 950 "                   |                                   |
| Comparative<br>Example 3 | "                                       | "                   | 18           | 1000 "                  |                                   |

TABLE 2—Continued

| fibers | dye | Addition amount (parts)<br>paper<br>strengthening<br>agent | fire<br>retardant | fixing agent | coagulating<br>agent |
|--------|-----|------------------------------------------------------------|-------------------|--------------|----------------------|
|--------|-----|------------------------------------------------------------|-------------------|--------------|----------------------|

## Example 3

Note:  
N.B.K., bleached sulfate pulp of soft wood  
SR drainage rate

The embodiments of the invention in which an exclusive property or privilege is claimed are defined as follows:

1. In a loudspeaker of the type which comprises a speaker diaphragm or cone adapted to generate sonic and/or subsonic vibrations in response to an electrical signal, the improvement which comprises: said diaphragm or speaker cone is made of cellulose fiber paper containing uniformly distributed therein (1) from 10 to 50 parts by weight of particles of chlorinated polyolefin having a molecular weight of from 500 to 40,000 and a chlorine content of from 40 to 75 percent by weight and (2) from 5 and 40 parts by weight of particles of antimony trioxide, the amounts of (1) and (2) each being based on 100 parts by weight of cellulosic fibers, whereby said diaphragm or speaker cone is non-flammable.

2. A loudspeaker as claimed in claim 1, in which the particles of (1) and (2) each having a particle size in the range of from 80 mesh to 300 mesh.

3. A loudspeaker as claimed in claim 2, in which the amount of (1) is 20 to 40 parts by weight and the amount of (2) is 10 to 30 parts by weight, each per 100 parts by weight of fibers.

4. A loudspeaker as claimed in claim 1, in which the paper also contains (3) 0.1 to 5 parts by weight of paper strengthening agent, (4) 1 to 5 parts by weight of fixing agent, and (5) 0.01 to 0.1 part by weight of coagulating agent, each per 100 parts by weight of fibers.

5. A loudspeaker according to claim 1 wherein said chlorinated polyolefin is chlorinated polypropylene.

6. A loudspeaker according to claim 1 wherein said chlorinated polyolefin is chlorinated polyethylene.

7. A loudspeaker according to claim 1 wherein said chlorinated polyolefin is chlorinated natural or synthetic rubber.

8. A loudspeaker according to claim 1 wherein said chlorinated polyolefin is a mixture comprising at least two components selected from the group consisting of chlorinated polyethylene, chlorinated polypropylene and chlorinated natural or synthetic rubber.

9. In a loudspeaker of the type which comprises a speaker diaphragm or cone adapted to generate sonic and/or subsonic vibrations in response to an electrical signal, the improvement which comprises: said diaphragm or speaker cone is made of cellulose fiber paper containing uniformly distributed therein (1)

from 10 to 50 parts by weight of particles of bromine containing chlorinated polyolefin having a molecular weight of from 500 to 40,000, a chlorine content of from 10 to 30 percent by weight and a bromine content of from 60 to 80 percent by weight, and (2) from 5 to 40 parts by weight of particles of antimony trioxide, the amounts of (1) and (2) each being based on 100 parts by weight of cellulosic fibers, whereby said diaphragm or speaker cone is nonflammable.

\* \* \* \* \*

40

45

50

55

60

65

UNITED STATES PATENT AND TRADEMARK OFFICE  
CERTIFICATE OF CORRECTION

PATENT NO. : 3 907 063  
DATED : September 23, 1975

INVENTOR(S) : Masahiko Nakazawa et al

It is certified that error appears in the above-identified patent and that said Letters Patent are hereby corrected as shown below:

Column 9, line 23; change "5 and 40" to ---5 to 40---.

Signed and Sealed this  
twentieth Day of January 1976

[SEAL]

Attest:

**RUTH C. MASON**  
*Attesting Officer*

**C. MARSHALL DANN**  
*Commissioner of Patents and Trademarks*